

3,658,975

## PROCESS FOR THE PRODUCTION OF POLYAMIDE CASTINGS

Jan Drabek, Oto Horak, Zdenek Ditych, and Svatoslav Záhorovský, Pardubice, Czechoslovakia, assignors to Výzkumný ústav syntetických průmyslových a laku, Pardubice, Czechoslovakia  
No Drawing. Filed Sept. 11, 1969, Ser. No. 857,204  
Claims priority, application Czechoslovakia, Sept. 11, 1968, 6,359/68, 6,366/68; Aug. 11, 1969, 5,559/69  
Int. Cl. B21d 39/00; B29c 1/12; B29d 3/00  
U.S. Cl. 264—94 10 Claims

### ABSTRACT OF THE DISCLOSURE

A process for the production of polyamide castings, containing cavities or fitted with a metal shaft, by an activated anionic polymerization of lactams in a mould, the mould being fitted with a composite core or metal shaft, the core or metal shaft having an outer inflatable jacket prepared by winding an elastic tube around the inner core or metal shaft with neighboring turns in engagement, inserting the composite core or metal shaft into a preheated stationary mould, inflating the tube with compressed gas, filling the mould with a lactam melt containing an alkaline catalyst, promoter, and/or pigments, and/or fillers, and/or other additives, the lactam melt then being polymerized at a temperature lower than the melting point of the polylactam formed, and after cooling, the composite core including said outer inflatable jacket is removed from the finished casting to give a casting with a cavity or in which the metal shaft together with the outer inflatable jacket remains tightly gripped in the casting.

The invention relates to a new process for the production of polyamide castings containing cavities or fitted with a metal shaft which comprises an activated anionic polymerization of a lactam or a mixture of lactams in a mould. Prior to the actual polymerization, the core or the metal shaft is provided with an outer inflatable jacket prepared by winding an elastic tube around the inner core or metal shaft with neighboring turns in engagement. When producing castings containing cavities, the composite core is removed after polymerization and cooling of the casting. In castings fitted with a metal shaft, the metal shaft remains together with the outer inflatable jacket tightly gripped by the casting. In both cases the high shrinkage stress ordinarily resulting in cracks of the castings is eliminated.

When producing polyamide castings containing cavities by casting melted lactam in the presence of an alkali catalyst and promoter directly on metal cores, followed by polymerization, the considerable shrinkage of castings during polymerization followed by cooling from polymerization temperature to room temperature is a cause of many disadvantages. The total volume shrinkage amounts to approximately 15%, linear shrinkage being about 4-5%. As the thermal dilatation of the metal core is approximately one order lower for the difference between the polymerization temperature and room temperature, e.g. steel 0.2%, the casting grips the core so tightly that it cannot be removed. The casting may even break (crack), if the strain caused by this shrinkage is higher than the tensile strength of polyamide. For this reason it is usually necessary to bore the desired hole in the finished casting, which means a loss of material as well as further drilling costs. Aside from this, the solid casting must be cooled very slowly, while

castings containing holes may be cooled much more rapidly. The danger of internal stress is much less in castings containing holes than in solid castings having no holes.

During the production of castings containing a metal shaft, e.g. calender bowls and gear-wheels, such high stresses are formed that the castings nearly always crack, and such cracking cannot be prevented even by long-time tempering. Therefore it is necessary to produce casting containing a metal shaft in such manner that in the first stage a solid casting from alkali polymerized lactam is produced. A hole is then formed in this solid casting by mechanical means, which hole may be fitted with slots. The casting worked in this way is warmed and then attached to the shaft. This procedure is expensive and lengthy. German Pat. No. 1,214,865 describes the production of calender bowls coated with a layer of alkali polymerized lactams by rotational casting, which process removes the shrinkage of the casting in the direction towards the metal shaft. But since the process requires a centrifugal acceleration of at least 500 g, and the axial shrinkage of the surface is eliminated by the position of the rotation axis, the requirements for machinery equipment are very high. According to U.S. Pat. No. 3,184,828 the effect of shrinkage during the production of calender bowls from alkaline polymerized lactams is eliminated by a deformable metal jacket on the shaft of the calender bowl, while either the shaft is fitted with axial slots and the jacket has a circular cross-section or the metal jacket having axial slots or ribs is fitted on the shaft, which has a circular cross-section. The sealing of the axial cavities thus formed on the shaft towards the mould is not solved by this patent, although the success of the process is totally dependent on it, because if the lactam melt poured into the mould penetrates into these cavities, then the effect of the deformable jacket is nullified. Aside from this difficulty, the production of the deformable metal jacket is complicated and expensive.

All the deficiencies set forth above are obviated by the present invention, which relates to a process for the production of polyamide castings containing cavities or fitted with a metal shaft by the process of using an activated anionic polymerization of lactams in a mould containing a composite core or a metal shaft. According to the present invention the core or metal shaft is provided with an outer inflatable jacket prepared by winding an elastic tube around the inner core or metal shaft with neighboring turns in engagement. The tube is inflated with compressed gas, and said composite core or metal shaft is inserted into a preheated stationary mould, the mould is then filled with melted lactam or a mixture of lactams containing an alkali catalyst, promoter, and optionally pigments and/or fillers and/or other additives. This reaction mixture is polymerized at a temperature lower than the melting point of the polylactam formed thereby. After cooling, the composite core including the outer inflatable jacket is removed from the casting to give a casting with a cavity or the tightly gripped metal shaft together with the outer inflatable jacket is allowed to remain in the casting.

The elastic tube used for the production of the outer inflatable jacket is made from a thermostable macromolecular material, such as silicone rubber.

When producing castings containing cavities a pressure is formed in said elastic tube before the beginning of the polymerization, which is kept there during the polymerization and is released during or after cooling of the casting. During the production of castings containing a metal shaft, the pressure formed in the elastic tube is progressively lowered during the polymerization and the cooling is carried out simultaneously with and according to the shrinkage of the casting. The pressure in the elastic tube is exerted by air compressed to 1-20 atm.

The stationary mould used in the process of the invention is made of metal and preheated to a temperature of 120–200° C., preferably 130–160° C. The melt of lactam or mixture of lactams is heated to a temperature of 80–180° C., preferably 120–150° C. 6-caprolactam or its mixture with  $\omega$ -laurolactam are the lactams most frequently and preferably used for the purpose of the present invention. The polymerization is effected in the presence of 0.1–2 mole percent, preferably 0.25–0.4 mole percent, of an alkaline catalyst, which is preferably an alkaline salt of a lactam, such as the sodium salt of 6-caprolactam. The polymerization is accelerated by the addition of 0.05–5 mole percent, preferably 0.25–0.5 mole percent, of a promoter, preferably an acyl compound, such as N-acetyl-6-caprolactam, or an isocyanate, such as hexamethylene-1,6-diisocyanate or triphenylmethane-4,4',4"-triisocyanate.

The present process for the production of castings from alkaline activated polyamide as disclosed and claimed herein offers a number of advantages in comparison with processes known before. Castings containing transverse or blind holes can be produced by direct casting into moulds containing cores. There is no danger of high internal stresses being formed and removal of the cores from the castings is much easier. The influence of shrinkage can be eliminated in any required direction, particularly by the use of the inflatable hollow jackets, held under excess pressure as described herein.

The castings fitted with a metal shaft are produced according to the present invention by a single operation in contrast to the three operations necessary for the known and previously used procedures, i.e. production of the casting, mechanical working by boring a hole therein, followed by fitting the worked casting onto a metal shaft. The production by the present invention does not require any complicated equipment such as is necessary for rotation casting. The process according to the invention facilitates the production of polyamide castings fitted with a metal shaft with a reproducible tension, by which the casting grips the metal shaft, depending on the tangential forces, which the metal shaft has to transmit onto the casting.

6-caprolactam is the most frequently used and most desirable lactam for the process according to the invention. Examples of other lactams suitable for the alkaline activated polymerization are enantholactam, caprylolactam, laurolactam, and lower lactams such as those of 2-pyrrolidone, 2-piperidone and also beta-lactams, such as beta-propiolactam, which cannot be polymerized hydrolytically. To modify the properties of polylactams, copolymers or mixtures of lactams are possible, such as 6-caprolactam admixed with C-alkyl-6-caprolactam or  $\omega$ -laurolactam.

The alkaline activated polymerization of these lactams is most often activated by alkaline reacting substances (alkali metals, alkaline earth metals or the hydrides, oxides, hydroxides, alcohols, amides, salts, and other derivatives thereof), Grignard reagents, and organometallic compounds. The most important catalyst is an alkaline salt of a lactam, such as the sodium salt of 6-caprolactam, which may be added to the lactam reaction mixture either directly or may be formed before the beginning of the polymerization in situ. The amount of initiators can vary from about 0.1 to about 2 mole percent, preferably from 0.25 to 0.4 mole percent, the amount being based on the lactam or mixture of lactams being polymerized.

Examples of the preferred promoters are the acyl compounds (N-acyllactams, N,N'-diacyl-bis-lactams, cyclic imides of dicarboxylic acids, and the like) and the isocyanates (butylisocyanate, hexamethylene-1,6-diisocyanate, tolylendiisocyanates, 4,4'-diphenylmethanediisocyanate, triphenylmethane-4,4',4"-triisocyanate, and the like). Other suitable and useful activators are carbodiimides, anhydrides, chlorides, hydrazides, amides, and esters of acids, lactones, imines, substituted ureas, nitrogenous, heterocyclic and other compounds, and various ethers and ke-

tones. The amount thereof required for promoter usage varies from about 0.05 to about 5 mole percent, preferably from 0.25 to 0.4 mole percent, based on the lactam or mixture of lactams being polymerized. The useful promoters can be used either separately or as a mixture or can be formed in situ in the course of the polymerization. Most frequently used promoters are the N-acyllactams, particularly N-acetyl-6-caprolactam.

To control the course of the polymerization process, it is possible and may be desirable to add a third component into the catalyst and promoter system, for example an alcohol, phenol or amine, which prolongs the catalytic effect of the system and controls the value and distribution of the medium molecular weight of the polylactams.

It is possible to add optionally reinforcing and non-reinforcing fillers and pigments (glass, asbestos, metal, cellulose and synthetic fiber materials, metal salts and oxides, metallic powders, carbon black, graphite, cement, silica, cadmium, zinc sulphide, molybdenum sulphide, various macromolecular substances, such as polyolefins, polytetrafluoroethylene, and the like). Furthermore, it is also possible to include such known additives as stabilizers, lubricants, plasticizers, blowing agents, solvents, surface active agents, and the like.

Substantially sealed moulds, made of material thermally stable up to 250° C., are suitable for the production of the castings according to the present invention. Particularly convenient are aluminum and aluminum alloys, nickel and chromium. It is also possible to use ceramic or laminated moulds and the like. Into the mould there are inserted suitable cores, preferably made of metal, or a metal shaft, usually made of steel.

The composite cores or metal shafts used in accordance with the present invention are provided with an outer jacket made of an elastic inflatable tube prepared from an elastic material, which is capable of withstanding temperatures up to about 200° C., which does not affect the polymerization of the lactam unfavorably and which does not have an affinity for the reaction mixture. It is possible to use thermostable macromolecular materials, such as silicone rubber, fluoroplastics, polyimides, polysulphones, thermostable, synthetic rubbers, and the like. A pressure of 1–20 atm., preferably 1–5 atm., is produced in the elastic tube before start of the polymerization by compressed gas, usually and preferably air. The pressure depends on dimensions and properties of the outer inflatable jacket as well as on dimensions and properties of the polyamide castings.

The production of polyamide castings according to the present invention is usually carried out in the following manner:

A composite core of metal shaft, equipped with an outer inflatable jacket, made of elastic tubes, is inserted into a stationary mould. The elastic tube is inflated by gas to a suitable pressure. The lower part of the mould, containing the composite core or the metal shaft, is substantially and carefully sealed, its upper part is closed by a loose cover. The mould containing the composite core or metal shaft is placed into appropriate heating equipment and is warmed to the desired temperature. A mixture melt containing a lactam or a mixture of lactams, an alkaline catalyst, a promoter and other additives, if and as desired, is poured through a filling tube inserted in the cover and reaching to the bottom of the mould. After the mould is filled, the filling tube is removed and the temperature in the heating equipment is raised to the selected and appropriate polymerization temperature.

The polymerization is effected during a period of 15–30 minutes. Then the mould, containing the casting is allowed to cool gradually to room temperature. After cooling, it is removed from the heating equipment, the cover of the mould is removed and the polyamide casting is taken out. When castings containing cavities are produced, the pressure is removed from the elastic tube and the composite core is extracted together with the outer inflatable jacket.

When producing castings containing a metal shaft, the pressure in the elastic tube is gradually lowered during the polymerization and the cooling is effected according to the shrinking characteristics of the casting. The casting grips the metal shaft firmly together with the outer inflatable jacket.

The present invention facilitates the production of castings made of polyamides produced by anionic activated polymerization, containing one or more cavities or metal shafts. The invention process can be used for the production of bearings, linings, propellers, carrying rollers, cams, flanges, packings and the like. The process according to the invention is well adapted for the production of rolls covered by a polyamide layer for textile, paper, tanning and printing machines. In these applications the outstanding properties of polyamides, such as retention of shape at high temperatures, high abrasion resistance, non-sensitivity to passage of flashes, and the like, find extensive utilization. Other applications are in the production of large gears, trolley wheels for cranes, cableways and similar, i.e. in any instance or circumstance where it is necessary to transmit forces from the shaft to the polyamide casting and at the same time utilize the outstanding properties of polyamides.

The following examples are given only for the purpose of illustrating the present invention, wherein ° stands for ° C., and % for mole percents unless otherwise indicated.

#### EXAMPLE I

Two cores around which elastic tubes made of a silicone rubber of 1 mm. thickness were previously wound with neighboring turns in engagement are fitted by means of screws to the mould. These tubes had been previously blinded on one end by cold curable silicone rubber and the first turn (containing the blinded end) was glued by the same material at the face of the cores. A similar method was used at the last turn (at the walls of the mould) and the inlets of compressed air were introduced into both tubes through the openings in the wall of the mould and sealed in these openings by cold curable silicone rubber. The mould is loosely closed by a cover through the openings of which the filling tube is inserted into the mould. The mould assembled in this way is put into the heating equipment and heated to a temperature of  $135 \pm 5$ °. Both tubes are inflated through the inlets by compressed air in such a way, that the outer dimensions of the jacket formed by these are at least 6-8% greater than the corresponding dimensions of the core increased by a quadruple of the thickness of the walls of the tube. The mould is then filled with anhydrous 6-caprolactam,  $125 \pm 5$ ° warm, containing 0.50% of the potassium salt of 6-caprolactam and 0.18% of hexamethylene-1,6-diisocyanate. After the mould is filled, the filling tube is removed and the temperature in the heating equipment is raised to  $190 \pm 5$ ° during 15 minutes. Afterwards the mould is let to cool during 36 hours to about 20°. About 1 hour after the end of the polymerization, the excess pressure from the tubes is released. After cooling to about 20°, the mould containing the casting is taken out of the heating equipment and after unscrewing the screws and releasing the inlets of compressed air, the casting is taken out of the mould together with both cores and the tubes. The last step is the removing of both cores and tubes from the casting.

#### EXAMPLE II

Into a steel mould for casting a gearwheel there is inserted the metal shaft of this wheel. The metal shaft had been previously wound by a tube made of silicone rubber, so that the neighboring turns are in engagement. The lower part of the tube was blinded in advance by cold curable silicone rubber, its upper part being fixed on the metal shaft by a suitable clamp. The metal shaft, provided with the tube, is fixed in the steel mould by means of a packing made of silicone rubber. The steel mould is closed by a loosely placed cover, through which passes

the upper part of the wound elastic tube and the filling tube. The mould assembled in this way is warmed in suitable heating equipment to the temperature of  $135 \pm 5$ ° C., the wound elastic tube is filled with compressed air to a pressure of 1.5 atm. and through the filling tube, anhydrous 6-caprolactam, heated to  $125 \pm 5$ ° and containing 0.40% of the potassium salt of 6-caprolactam and 0.18% of hexamethylene-1,6-diisocyanate, is fed into the assembled steel mould. After the mould is filled, the filling tube is removed and the temperature of the heating equipment is raised to  $190 \pm 5$ ° C. during 15 minutes. The casting is then allowed to cool to a temperature of about 20° C. during 24 hours. After this period, the steel mould containing the casting is removed from the heating equipment and its cover is taken off together with the packing. The gear-wheel, joined firmly with the metal shaft and the wound tube, is taken out of the steel mould. All air has been expelled from the tube by shrinkage during polymerization and cooling, so that a firm joint between the metal shaft and the casting is obtained without causing such stress in the casting that it might be spontaneously damaged.

#### EXAMPLE III

The metal shaft of a calender bowl is connected by means of a sealing and a nut to a steel mould, open on top. The shaft is provided with a closely adhering jacket made of foamed silicone rubber ( $\epsilon = 0.5$  kg./dm.<sup>3</sup>) of 5 mm. thick. The mould containing the shaft is heated in a suitable heating equipment to the temperature of  $130 \pm 5$ ° C. Then a filling tube reaching up into the bottom is inserted and the mould is filled with the reaction mixture. This mixture contains 65% of anhydrous caprolactam and 35% of anhydrous laurolactam, heated to  $130 \pm 5$ ° C. and containing 0.33% of the lithium salt of 6-caprolactam and 0.15% of triphenylmethan-4,4',4''-triisocyanate. After the mould is filled, the filling tube is removed and the temperature of the heating equipment is raised during 15 minutes to  $180 \pm 5$ ° C. At the end of this heating period, the polymerization is complete and the mould containing the casting is allowed to cool to a temperature of 20-30° C. for 48 hours. The copolymer casting, joined firmly with the metal shaft by means of the compressed layer of foamed silicone rubber, use of which eliminates the influence of shrinkage during polymerization and cooling, is taken out.

#### EXAMPLE IV

The metal shaft of a calender bowl, provided with a closely fitting hollow jacket made of silicone rubber, the walls of which are 1 mm. thick and provided with an inlet tube for compressed air, is fixed in the mould by means of a gasket ring, made of silicone rubber, and a nut. The hollow jacket is joined with the gasket ring by a cold vulcanizable silicone rubber adhesive. A filling tube is introduced into the mold, the top of which is closed by a loosely placed cover. After the mould has been warmed in suitable heating equipment to the temperature of  $145 \pm 5$ ° C., the hollow jacket is filled with air, compressed to 1.2 atm. Then the mould is filled through the filling tube with anhydrous 6-caprolactam, heated to  $135 \pm 5$ ° C. and containing 0.35% of Na-salt of 6-caprolactam and 0.30% of N-acetyl-6-caprolactam. After the mould is filled, the filling tube is removed and the temperature of the heating equipment is raised to  $190 \pm 5$ ° C. during 20 minutes. After this period, during which the polymerization is completed, the mould containing the casting is allowed to cool to a temperature of 20° C. for 36 hours. After the cooling period, the mould containing the casting is taken from the heating equipment, the cover is removed and, after unscrewing the nut, the calender bowl is removed from the mould. The hollow jacket is compressed by the shrinkage during polymerization and cooling so that all air has been expelled from

the hollow jacket and there is only a layer of compressed silicone rubber between the metal shaft and the casting.

#### EXAMPLE V

Into a steel mould for casting a gear-wheel there is inserted the metal shaft of this wheel. The metal shaft had been previously wound by a tube made of silicone rubber. The lower part of the tube was blinded in advance by cold curable silicone rubber, its upper part being fixed on the metal shaft by a suitable clamp. The metal shaft, provided with the tube, is fixed in the steel mould by means of a packing made of silicone rubber. The steel mould is closed by a loosely placed cover, through which passes the upper part of the tube and the filling tube. The mould assembled in this way is warmed in suitable heating equipment to the temperature of  $135 \pm 5^\circ \text{C}$ ., the tube is filled with compressed air to a pressure of 1.5 atm. and through the filling tube, anhydrous 6-caprolactam, heated to  $125 \pm 5^\circ \text{C}$ . and containing 0.40% of the potassium salt of 6-caprolactam and 0.18% of hexamethylene-1,6-diisocyanate, is fed into the assembled steel mould. After the mould is filled, the filling tube is removed and the temperature of the heating equipment is raised to  $190 \pm 5^\circ \text{C}$ . during 15 minutes. The casting is then allowed to cool to a temperature of about  $20^\circ \text{C}$ . during 24 hours. After this period, the steel mould containing the casting is removed from the heating equipment and its cover is taken off together with the packing. The gear-wheel, joined firmly with the metal shaft, is taken out of the steel mould. All air has been expelled from the tube by shrinkage during polymerization and cooling, so that a firm joint between the metal shaft and the casting is obtained without causing such stress in the casting that it would be spontaneously damaged.

What is claimed is:

1. In a process for the production of polyamide castings, containing cavities or fitted with a metal shaft, said polyamide being the product of activated anionic polymerization of lactams in a mould, the improvement which comprises fitting said mould with a composite core or metal shaft provided with an outer inflatable jacket prepared by winding an elastic tube around the inner core or metal shaft with neighboring turns in engagement, inserting said composite core or metal shaft into a pre-heated stationary mould, inflating said elastic tube with compressed gas, filling said mould containing said composite core or metal shaft with a melted mixture containing a lactam or a mixture of lactams, an alkaline

catalyst, promoter and optionally pigments and/or fillers and/or other additives, polymerizing said mixture at a temperature lower than the melting point of the poly-lactam formed, and cooling the resulting casting.

5 2. A process according to claim 1, comprising after cooling, removing the composite core including said outer inflatable jacket from said casting to give a casting with a cavity.

10 3. A process according to claim 1, comprising after cooling, allowing the tightly-tripped metal shaft together with the outer inflatable jacket to remain in said casting.

4. A process according to claim 1, wherein said elastic tube is made of a thermostable macromolecular material.

15 5. A process according to claim 1, wherein said elastic tube is made of silicone rubber.

6. A process according to claim 1, wherein during the production of castings containing cavities, a pressure is formed in said elastic tube before the polymerization and said pressure is maintained during the polymerization.

20 7. A process according to claim 6, wherein the pressure is released during cooling of the casting.

8. A process according to claim 6, wherein the pressure is released after cooling of the casting.

9. A process according to claim 1 wherein during the 25 production of castings fitted with a metal shaft, the pressure formed in the elastic tube is progressively lowered during the polymerization and cooling in controlled accordance with the shrinkage of the casting.

10. A process according to claim 1, wherein the pressure in the elastic tube is exerted by air, compressed to 30 1-20 atmospheres.

#### References Cited

##### UNITED STATES PATENTS

|           |         |                          |         |
|-----------|---------|--------------------------|---------|
| 3,135,640 | 6/1964  | Kepka et al. -----       | 264—314 |
| 3,177,105 | 4/1965  | Wiltshire -----          | 264—314 |
| 3,222,443 | 12/1965 | Dames, Jr., et al. ----- | 264—331 |
| 3,470,199 | 9/1969  | Jung -----               | 264—310 |
| 3,493,647 | 2/1970  | Schuette et al. -----    | 264—331 |

##### FOREIGN PATENTS

|           |        |              |         |
|-----------|--------|--------------|---------|
| 1,520,770 | 4/1968 | France ----- | 264—314 |
|-----------|--------|--------------|---------|

ROBERT F. WHITE, Primary Examiner

J. R. THURLOW, Assistant Examiner

##### U.S. CL. X.R.

29—452; 260—78 L; 264—266, 314, 331